

## UNITED STATES PATENT OFFICE

2,035,394

## CAST STEEL

Russell H. McCarroll and Gosta Vennerholm,  
Dearborn, Mich., assignors to Ford Motor Company,  
Dearborn, Mich., a corporation of Delaware

No Drawing. Application February 9, 1934,  
Serial No. 710,524

2 Claims. (Cl. 75—125)

This invention relates to a new and improved steel alloy having new and exceptional properties and capable of being employed for the casting of many articles of manufacture for which no known alloys or metals could be satisfactorily employed. In the fabrication of certain automobile parts it was found desirable to use a casting with relatively thin walls to which was to be integrally united metal tubing. The growth and improvement of welding practice has made the use of welded joints more common because of facility for production methods. While ordinary cast steel lends itself to welding, it cannot be satisfactorily successfully used for very thin wall or intricate castings due to lack of sufficient fluidity. Also because of the greater cost of making an ordinary steel casting of such a design it would be prohibitive, if in fact it were possible to secure sound castings in ordinary steel of such a design. Malleable iron is especially well adapted for thin castings but cannot be welded satisfactorily because of its tendency to harden and become brittle under the high heats of the welding operation which are above the critical temperature and because of the tendency of the free temper carbon content to oxidize and form gases which produce blow holes and thereby weaken the weld. Ordinary grey cast iron could not be successfully employed for articles of the type under consideration because of its relatively low physical properties and because high carbon content thereof results in marked hardening and embrittlement of the metal in the region of the weld after welding. The present invention has for its principal object to provide a new and improved steel alloy capable of being successfully cast to form thin walled castings and withstanding the high temperatures of welding operations without hardening effect or embrittlement and which, moreover, can be manufactured and fabricated at a relatively low cost.

We have found after considerable experimentation that a steel having an analysis falling within the following limits, will have all of the desired properties and none of the objectionable features as above set forth, of the more commonly used materials:

|      |                 |
|------|-----------------|
| 50 C | 0.25% (maximum) |
| Mn   | 0.15 to 0.65%   |
| Si   | 0.75% to 1.25%  |
| Cu   | 0.90 to 1.75%   |
| Fe   | balance         |

If desired sulphur up to 0.15 may be added for increasing ease of machineability.

It has been found that the presence of more than 0.25 C. results in a hardening and embrittlement of the metal in the region of the weld after the metal is subjected to the high welding temperatures.

The relatively high silicon content together with the copper results in increased fluidity which enables very thin wall castings to be satisfactorily produced. The silicon or copper contents in properly combined proportions give a lower melting point which tends to improve the welding properties of the metal. It is found that the silicon and copper go into solid solution with the iron to produce an alloy having excellent high physical properties; the high silicon content being important in this respect as it tends to increase the solubility of the copper, the metal having a tensile strength of from 85 to 90 thousand pounds per square inch and a Brinnell hardness of about 150.

While the silicon content should be kept high enough to secure the desired fluidity, it has been found to be best not to have an amount in excess of 1.25%, because of its effect on machineability especially in combination with a relatively high copper content.

It has also been found advisable not to have the copper content greater than 1.75%, thereby to avoid the tendency towards excessive air hardening.

The metal may be cast in green sand molds thus enabling savings to be effected in production costs. After casting an ordinary normalizing treatment is desirable, such normalizing resulting in a decided improvement in the physical properties by producing a marked grain refinement of the metal.

Although copper is employed, the copper content is relatively small, and the production cost of the metal is appreciably lower than that of either cast steel or ordinary malleable iron and possesses marked advantages over either in that it may be used for producing excellent thin wall castings, to which other parts may be integrally secured by welding; a strong welded joint being secured without producing any deterioration of the physical properties of the metal.

Although the invention has been described from the standpoint of its advantages when used for the manufacture of thin wall castings, to which it is desired to weld other parts, it will be understood that the invention is not to be considered as limited to this one specific use, but that as other uses will be readily apparent to the

skilled metallurgist and those in the art to which the invention appertains, it is the purpose to include herein such other uses.

We claim:

5 1. An article of manufacture a sound thin wall casting of low carbon, high silicon steel and having an analysis lying within the following limits:

C----- 0.25% (maximum)

Mn----- 0.15 to 0.65%

Si----- 0.75 to 1.25%

Cu----- 0.90 to 1.75%

Fe----- balance

10 19 Mn----- 0.15 to 0.65%

Si----- 0.75 to 1.25%

Cu----- 0.90 to 1.75%

Balance substantially all iron.

15 2. An article of manufacture comprising a sound thin wall casting of low carbon, high silicon

steel capable of withstanding welding temperatures without deterioration or air hardening effects, said steel having an analysis lying between the following limits:

C----- 0.25% (maximum) 5

Mn----- 0.15 to 0.65%

Si----- 0.75 to 1.25%

Cu----- 0.90 to 1.75%

Fe----- balance 10

and in which the silicon and copper contents are combined in approximately the proportions of 4 to 5 respectively.

RUSSELL H. McCARROLL,  
GOSTA VENNERHOLM.

15